

## UNITED STATES PATENT OFFICE

2,246,059

## COMPOSITION OF MATTER

Robert C. Moran, Wenonah, William L. Evers,  
Moorestown, and Everett W. Fuller, Wood-  
bury, N. J., assignors to Socony-Vacuum Oil  
Company, Incorporated, New York, N. Y., a cor-  
poration of New York

No Drawing. Application February 1, 1940,  
Serial No. 316,778

4 Claims. (Cl. 252—53)

This invention is directed to the stabilization of hydrocarbon oils of higher boiling points against the deteriorating effects of oxidation. Highly refined oils of the non-sludging types, such as the white oils, turbine oils, and the like, must be able to withstand the conditions of their use without the formation of acidic constituents of a corrosive or otherwise damaging nature. This invention contemplates the stabilization of such oils. Moderately refined oils of the nature of many lubricant fractions must likewise be able to withstand the conditions of their use without the formation of sludges, loss of color, or development of oxidation products corrosive to commonly used metals, as for instance to copper. This invention likewise contemplates the stabilization of such moderately refined oils. In short, this invention is directed to the stabilization against deterioration due to oxidation reactions of any petroleum fractions of a light lubricant nature or heavier, from the lightest spindle oils, through the various classes of moderately refined oils of higher viscosity, and inclusive of the highly refined oils such as turbine oils, white oils, and the like.

This invention has for an important object the preparation of oils falling within the above classes which are stable against oxidation and capable of meeting the normal conditions of their use without the formation of gummy material, sludges, materials of an acidic or corrosive nature, and/or darker color. It also has for an object the provision of a class of stabilizing materials not heretofore known to be effective for that purpose.

Recent changes in automotive engine design, tending toward higher bearing pressures, higher rotative speeds, higher engine temperatures, and the like, have occasioned departure from the use of the usual bearing metals such as Babbitt. The newer bearing metals are of different nature, and, while harder, are in general more susceptible to destructive agencies of a corrosive nature. Typical of these newer bearings are those composed of a cadmium-silver alloy supported upon a steel back, which are now widely installed in certain makes of automobiles. Others of these relatively new bearing metals which may be mentioned are cadmium-nickel and copper-lead alloys.

These changes in engine design have been concurrent with marked advances in methods of refining lubricant oils for automotive use. The demand for oils having lesser changes in viscosity with temperature change: i. e., higher viscosity index (V. I.), has been met by refining lubricants intended for motor oils by certain solvent-refining or solvent-extraction processes, wherein advantage is taken of the selective solvent power for hydrocarbons of various types which is possessed by certain liquid reagents—for example, dichlorodethyl ether, cresylic acid, phenol, chloraniline, chlorophenol, phenetidine, benzyl alcohol, nitrobenzene, benzonitrile, furfural, aniline, benzyl acetate, liquid sulfur dioxide, mixtures of liquid sulfur dioxide or aniline with benzol, and the like. These solvent-refining processes are operated to concentrate in the desired lubricant fraction those compounds of a "paraffinic" nature possessed of the ability to suffer only a small change of viscosity upon change of temperature, and to reject the compounds of "naphthenic" nature which do suffer such change of viscosity to a more marked degree. These refining processes have enabled supply of an oil of quite desirable general characteristics, definitely far superior to any oil previously produced from mixed base or asphaltic crudes, and superior to a like, though lesser, degree over oils previously produced from paraffin base crudes.

It has been found that the solvent-refined motor oils referred to above are for some reason definitely corrosive to the newer bearing metals under normal conditions of automotive use, sometimes resulting in bearing failure after only a few thousand miles of normal driving. It is further known that the same reaction, viz., corrosion of alloy bearing metals such as cadmium-silver, occurs in good paraffinic base oils which have not been subjected to solvent-refining. The higher the V. I. of the lubricating oil, the more pronounced is the tendency to corrosion of the kind referred to above; generally speaking, the problem is encountered in oils having a V. I. of 75 or higher, and becomes important in oils having a V. I. of 80 to 85 or higher, and very important in oils of 100 V. I. or higher.

It is an important object of this invention to provide means for satisfactorily inhibiting or

preventing this corrosion from taking place to a serious degree. It is an object of this invention to alter or modify a highly refined motor oil, normally corrosive, by the use of an additive ingredient capable of substantially inhibiting this corrosion. It is an object to provide a substantially non-corrosive motor oil of high V. I. An object of this invention is to provide an additive reagent or ingredient capable of inhibiting the corrosive properties of these oils. The production of solvent-refined oils of low corrosive properties under conditions of automotive use is a major object of this invention, as well as the method of production of such oils which couple high viscosity index with low tendency to corrosion.

We have found that hydrocarbon oils of the classes defined above can be stabilized in the respects above indicated by the addition thereto of small amounts of compounds selected from the class of aryl phosphites having the general formula  $(ArO)_3P$ , in which Ar designates an aryl radical, as for instance  $C_6H_5$  or  $CH_3C_6H_5$ . The aryl phosphites which are suitable for the uses of this invention are as follows: Compounds 25 of the general formula



where one or more of the R's is a radical selected from the group consisting of



where the R's are radicals selected from the group consisting of hydrogen, alkyl, hydroxy, halogen, aryl (such as phenyl and hydroxyphenyl), alkaryl, alkoxy, nitro, and amino and substituted amino (as phenyl or benzyl substituted). Of the above-defined classes of compounds, those at present preferred for the uses of this invention are those wherein all three R's are radicals of either type (a) or (b) defined above, and wherein the R's are either hydrogen or alkyl. Examples of specific materials which we have found especially suitable for the uses of this invention are triphenyl phosphite, tricresyl phosphites, and tribeta-naphthyl phosphite. Where R' is alkyl, it may range from a short alkyl such as methyl to very long alkyls corresponding, for example, to paraffin wax.

The general inventive concept as set forth in the preceding paragraph is embodied in our co-pending application Serial No. 106,227, of which the present application is a continuation in part. This application is specifically directed to that class of the aforesaid compounds in which R' is a long chain alkyl group corresponding to aliphatic hydrocarbons of the type characterizing paraffin wax. These compounds, which we may designate as wax-aryl phosphites, distinguish over the general class of phosphites described above in that they are effective to reduce the pour point of viscous mineral oil fractions in addition to

improving the oil in the aforesaid respects. Thus, the wax or heavy alkyl-substituted aryl phosphites are multifunctional oil-addition agents, functioning as pour depressants and oxidation inhibitors while the aforesaid general class of aryl phosphites possess as their common property that of corrosion or oxidation inhibition.

The specific compounds contemplated herein may be represented by the general formula



10 15 in which R represents a radical selected from the group consisting of hydrogen and the radicals



30 35 wherein at least one R' is a long chain alkyl radical corresponding to paraffin wax and the remaining R's are radicals selected from the group consisting of hydrogen, alkyl, hydroxy, aryl, alkaryl, alkoxy, nitro, amino, and substituted amino radicals, at least one of the R's being selected from the aforesaid group of radicals (a), (b) and (c). Of the compounds corresponding to the foregoing general formula preference is given to compounds of the type in which all of the R's are substituted with aryl radicals, at least 40 one of which has a long chain alkyl substituent corresponding to an aliphatic hydrocarbon group of the type characterizing paraffin wax. Such preferred compounds may be identified as triaryl phosphites in which at least one of the aryl radicals has at least one relatively long alkyl substituent of the general order corresponding to paraffin wax.

45 50 Triaryl phosphites of the character discussed above in which the aryl radical is derived from phenol may be represented by the general formula



55 60 65 70 75 80 85 90 95 100 wherein at least one R' is a long chain alkyl radical corresponding to the alkyl radicals characterizing paraffin wax and the remaining R's are radicals selected from the group consisting of hydrogen and alkyl.

These wax-aryl phosphites may be formed by first reacting a chlorinated paraffin wax or similar long chain aliphatic compound or predominantly aliphatic material with a hydroxyaromatic compound, such as phenol, naphthol, and the like, in the presence of a Friedel-Crafts catalyst to form a "wax-substituted phenol" or "wax-phenol" and then reacting the wax-phenol thus obtained with phosphorus trichloride.

For example, a so-called "monowax" phenol may be obtained by reacting a quantity of chlorinated paraffin wax (about 14 per cent chlorine content) with phenol in the presence of aluminum chloride, the reaction mixture being proportioned so that there is one atomic proportion of chlorine present for each mol of phenol. By changing the ratio of the chlorwax to phenol in the reaction mixture so that there are two, three or four atomic proportions of chlorine to one mol of phenol, the so-called di-, tri-, and tetra-wax phenols are obtained. The Friedel-Crafts reaction for obtaining the wax-phenol is carried out at elevated temperature, preferably not to exceed 350° F.

The wax-phenol reacts with the  $\text{PCl}_3$  at elevated temperature (from 103° F. to 205° F.) with the evolution of  $\text{HCl}$  gas. The use of a solvent such as ethylene dichloride is desirable to reduce foaming. Following the reaction the mixture may be taken up in benzene containing a little fusel oil and washed with hot water, thereby hydrolyzing any chlorine of the  $\text{PCl}_3$  which has not been substituted with the wax-aryl nucleus. The solvent may then be distilled off to obtain the final product.

The effectiveness of the compounds contemplated herein as addition agents for viscous mineral oil fractions is demonstrated by the following examples.

#### EXAMPLE ONE

##### POUR POINT DEPRESSION

The oil used in this test was an S. A. E. 30 motor oil having an A. S. T. M. pour point of +20° F. Several blends of this oil were prepared with wax-phenyl phosphites of the type contemplated herein and the pour points of such blends are set forth in Table I below, wherein the various wax-phenyl phosphites are identified by the reactants used in their preparation.

Table I

| Addition agent                          | Per cent | A. S. T. M. pour point<br>°F. |
|-----------------------------------------|----------|-------------------------------|
| None                                    |          | +20                           |
| Monowax-phenol- $\text{PCl}_3$ compound | 1.0      | +20                           |
| Do                                      | 0.5      | -10                           |
| Diwax-phenol- $\text{PCl}_3$ compound   | 0.5      | -25                           |
| Do                                      | 0.25     | -10                           |
| Triwax-phenol- $\text{PCl}_3$ compound  | 0.25     | -20                           |

#### EXAMPLE TWO

##### CORROSION INHIBITION

The oil used in this test was an S. A. E. 20 motor oil having a specific gravity of 0.872, a flash point of 435° F., and a Saybolt viscosity of 318 seconds at 100° F. The test involved placing a section of a bearing containing a cadmium-silver alloy surface and weighing about 6 grams in a sample of the oil and heating the oil to a

temperature of 175° C. for 22 hours while bubbling a stream of air against the surface of the bearing. The loss in weight of the bearing is a measure of the amount of corrosion which has taken place. Samples of the oil with the addition agent ("Inhibited sample") were run comparatively with the blank oil, the results being indicated in Table II below.

Table II

| Addition agent                            | Per cent | Mg loss in weight |       |
|-------------------------------------------|----------|-------------------|-------|
|                                           |          | Inhibited sample  | Blank |
| Monowax-phenol- $\text{PCl}_3$ compound   | 0.5      | 3                 | 24    |
| Diwax-phenol- $\text{PCl}_3$ compound     | 0.5      | 2                 | 24    |
| Triwax-phenol- $\text{PCl}_3$ compound    | 0.5      | 1                 | 24    |
| Tetrahexa-phenol- $\text{PCl}_3$ compound | 0.5      | 3                 | 24    |

From the foregoing examples it will be seen that the "wax-aryl phosphites" contemplated herein are effective to reduce the pour point and retard the deleterious effects of oxidation when added in minor proportions to viscous mineral oil fractions.

The amount of addition agent to be used will vary with the nature of the oil to be stabilized and with the use to which it will be put. In general, effective stabilization and pour point depression will be obtained in the oils of the class herein discussed with not more than 2% of the wax-aryl phosphites, usually not more than 1%. For more common uses, effective stabilization and pour point depression may be obtained with amounts in the neighborhood of 0.05 per cent to 0.50 per cent of these compounds.

In the claims, where the term "hydrocarbon oils of relatively high boiling point" or the equivalent thereof is used, it is intended to mean any and include all hydrocarbon mineral oil products normally used as lubricants or for electrical insulating purposes. It includes oils with an S. U. V. of 50 seconds at 100° F. or higher or a flash point greater than 200° F. (Cleveland open cup). This term, in effect, is in contradistinction to gasolines, kerosenes, and the like.

As aforesaid, this application is a continuation in part of our copending application Serial No. 106,227, filed October 17, 1936, which application is, in turn, a division of application Serial No. 46,870, filed October 26, 1935, now issued as Patent No. 2,058,343 of October 20, 1936.

We claim:

1. As an antioxidant for petroleum hydrocarbon oil of boiling point higher than that of gasoline and kerosene, a triaryl phosphite in which at least one of the aryl radicals has at least one relatively long alkyl substituent of the general order corresponding to paraffin wax.

2. An improved mineral oil composition comprising a petroleum oil of relatively high boiling point normally tending to deteriorate by oxidation when heated and in admixture therewith a small proportion, sufficient to retard said deterioration and depress the pour point of the oil, of a triaryl phosphite in which at least one of the aryl radicals has at least one relatively long chain alkyl substituent of the general order corresponding to paraffin wax.

3. An improved mineral oil composition comprising a petroleum oil of relatively high boiling

point, having added thereto a minor proportion of a compound of the general formula



5

in which R represents a radical selected from the group consisting of hydrogen and the radicals

(a)



(b)



(c)



10

15

20

wherein at least one R' is a long chain alkyl radical corresponding to the aliphatic groups characterizing paraffin wax and the remaining R's are radicals selected from the group consisting of hydrogen, alkyl, hydroxy, halogen, aryl, alkaryl, 25 alkoxy, nitro, amino and substituted amino radicals, at least one of the R's being selected from the aforesaid group of radicals (a), (b) and (c).

4. An improved mineral oil composition comprising a petroleum oil of relatively high boiling 30

point having added thereto a minor proportion of a compound of the general formula



wherein at least one R' is a long chain alkyl radical corresponding to the aliphatic groups characterizing paraffin wax and the remaining R's are radicals selected from the group consisting of hydrogen, alkyl, hydroxy, halogen, aryl, alkaryl, alkoxy, nitro, amino, and substituted amino radicals.

ROBERT C. MORAN.  
WILLIAM L. EVERE. 25  
EVERETT W. FULLER.

CERTIFICATE OF CORRECTION.

Patent No. 2,246,059.

June 17, 1941.

ROBERT C. MORAN, ET AL.

It is hereby certified that error appears in the printed specification of the above numbered patent requiring correction as follows: Page 2, first column, line 53, and second column, lines 34 and 39, for "R's" read --R's--; page 4, first column, line 27, claim 3, for "R's" read --R's--; and that the said Letters Patent should be read with this correction therein that the same may conform to the record of the case in the Patent Office.

Signed and sealed this 6th day of January, A. D. 1942.

Henry Van Arsdale,

Acting Commissioner of Patents.

(Seal)